

# UNITED STATES PATENT OFFICE.

MICHAEL A. POPKESS, OF KANSAS CITY, MISSOURI, ASSIGNOR TO BITUMINIZED ROAD COMPANY, A CORPORATION OF ARIZONA.

## PAVEMENT AND PROCESS OF MAKING THE SAME.

1,220,682.

Specification of Letters Patent. Patented Mar. 27, 1917.

No Drawing.

Application filed September 15, 1916. Serial No. 120,373.

*To all whom it may concern:*

Be it known that I, MICHAEL A. POPKESS, a citizen of the United States, residing at Kansas City, in the county of Jackson and 5 State of Missouri, have invented new and useful Improvements in Pavements and Processes of Making the Same, of which the following is a specification.

This invention relates to paving material 10 and, particularly, to paving material of the type covered by Letters Patent No. 1,008,433, granted to me November 14th, 1911, and consists in certain modifications of the process and product set forth therein.

15 An important object of this invention is to provide a pavement which is substantially free from mineral particles large enough to fracture in use, which has a homogeneous wear resisting and traffic supporting body, which will present a dense, smooth and malleable surface, which is tough, tenacious and of maximum durability, which is practically free from voids, self-healing and easy to repair and which will 20 not ravel, "rut", wear into holes, flow, creep, nor push into waves.

Other objects and advantages of the invention will be apparent during the course of the following description.

30 In an application for Letters Patent filed by me April 21st, 1916, Serial No. 92,704, of which the present application is a division, I explained that I discovered in the use of the machine, disclosed in an application filed by me April 4, 1914, Serial No. 829,549, that the hard particles of dirty sand or gravel, decayed or soft stone, weathered rock and the like, are cleaned, polished 35 and fractured, and in such condition serve

40 as a valuable addition to the paving material set forth in my said patent. Application No. 92,704 covers the resulting paving material, that is to say, paving material composed of the earthy dust set forth in my 45 said patent, or any kind of mineral dust, intimately mixed with sufficient asphalt to form a non-flowing matrix, in combination with a filler of clean stony particles, embedded in and separated from each other by 50 such matrix, which pavement differs from previously known pavements, in that the

said filler is not the main wear resisting and traffic supporting ingredient but those functions are performed by the mixture of asphalt and mineral dust. In such prior 55 pavements the mineral aggregate of broken rock, or gravel, and sand was so proportioned and arranged as to give a structure having inherent stability, that is the bodies of mineral matter supported and held each 60 other, the asphalt functioning merely as a cement to hold them in place, and to waterproof the structure. In the type of pavement of said application, the asphalt and dust together form a hard but malleable 65 material which is the wear-resisting element of the roadway.

In the further course of experimentally treating such materials in the said machine, I found that the degree of pulverization of the rock, gravel, sand and the like, depends very largely upon the speed of rotation of the pulverizer and that it is possible, by speeding up the pulverizer, to reduce to dust a large proportion of such material and I discovered that the resulting mixture of stony dust thus obtained and earthy or clayey dust containing none or substantially free from the coarser particles will form a satisfactory wear resisting and 80 traffic supporting mass when mixed in the proper proportions with a suitable binder, preferably asphalt. I also discovered that other stony material, such as sand, gravel, rock, and the like, reduced to an impalpable 85 dust, even though free or substantially free from soil, loam, or clay dust, will also serve to form a suitable pavement when mixed in the proper proportions with a suitable binder, such as asphalt. 90

My present invention, which is founded upon these discoveries, consists in a pavement comprising mechanically pulverized stony material of the nature of silica and silicates such as sand, gravel, pebbles and 95 larger stones, rock, cinders and the like, in the form of impalpable dust, mixed in the proper proportions with a suitable binder, preferably a bituminous binder such as asphalt, and in its preferred embodiment my 100 invention consists in preparing a paving composition from such stony material, in

the form of dust, and disintegrated earthy material, such as soil, loam, or clay and the like, in the form of dust, the stony material and the earthy material being mixed in the proper proportions with a suitable binder. The invention also comprises the process of making such pavement. In this material the dustlike particles are too small to permit such, if any, mechanical locking engagement or mutual support as is the case with compositions using mineral aggregates of the usual type.

In the preferred practice of my process I subject the mineral material to be employed therein including both stony material alone, such as clean sand, gravel, rock and the like, and earthy material, if the latter is present therewith, as in the case of dirty sand or gravel, decayed stone, weathered rock and the like, to the action of pulverizing or disintegrating means such, for example, as the pulverizer of my said machine or any other suitable means, and, in this way, the stony particles are fractured and reduced to dust-like form and the larger particles are given sharp corners and edges observable under the microscope, in contra-distinction to the round corners and edges which are possessed by ordinary sand and gravel which has been disintegrated by nature. The result of subjecting the mineral material to such pulverizing action, which is preferably carried on until substantially all of the particles are reduced to the form of dust, is that in the product a natural grading of the various sized mineral particles takes place, that is to say, the spaces of voids between the larger particles are filled by the very fine dust. This obviates any necessity for artificial grading by weighing or measuring the materials of different sizes, to reduce the number of voids, a practice which is followed in the manufacture of ordinary asphalt pavements, made of sand, gravel or rock and asphalt. With such fine material there cannot, of course, be any voids of appreciable size between the particles; there cannot be the large voids which occur in the ordinary sand, rock and gravel asphalt pavements and which become filled with "lakes" of asphalt which soften and become displaced under heat.

The mineral material pulverized, or pulverized and disintegrated as described, is in the form of a very fine palpable dust, such that substantially all, or, at least, 90 per cent. will pass through a 30 mesh screen and 50 per cent. will pass through a 100 mesh screen; but I prefer to pulverize, or pulverize and disintegrate, the material to a degree of fineness such that 70 per cent. will pass through a 200 mesh screen.

In mixing the mineral dust, either pulverized stony material alone or such material mixed with disintegrated earthy material,

with the binder I may proceed in accordance with the customary practice in the paving art. Preferably however the mineral dust is heated and dried, either before it is disintegrated or while it is being disintegrated, or afterward, and is then mixed in that condition with the hot binder such as asphalt. The disintegrated material may, however, be mixed in a moist condition with the binder, natural or artificial heat being applied during or after the mixing so that the binder will penetrate the material as the moisture is driven off and replace such moisture as more particularly described in an application filed by me April 11, 1916, Serial No. 99,391. The proportion of binder which should be used depends upon the fineness of the mineral dust employed, the finer such dust the greater the percentage of binder being required. It also depends upon whether stony dust alone is used or stony dust and earthy dust, the former requiring less binder than the latter. Where both are present the greater the proportion of earthy material the greater percentage of binder required. In actual practice when using a bituminous binder, such as asphalt, I may employ from 12 to 25 per cent. of such binder. I prefer however to employ from 14 to 18 per cent. unless the material contains little or no earthy material, in which case I ordinarily employ from 12 to 16 per cent. of binder, the percentage set forth herein being calculated by weight but in actual practice the amounts can be measured or weighed.

In the use of my paving material it is spread upon a prepared base and tamped or rolled on the surface to be paved. It may however be pressed into blocks.

It will be understood that the term "dust" as herein employed refers to material of such an extreme degree of fineness that when dry it is dust-like. The term is not intended to refer only to dry material but is intended to include wet, moist and dry material as well, providing it is of the degree of fineness that renders it dust-like when dry.

While I have particularly set forth the preferred degree of fineness of the mineral dust and the proportions of binder to be employed with such material, it is to be understood that these may be varied somewhat without departing from the spirit of my invention or the scope of the subjoined claims. It is also to be understood that in some cases stony material can be obtained which is in the form of fine dust, and such dust can be used to produce a commercially practical pavement either alone or in conjunction with dust made by disintegrating earthy material such as soil, loam, clay or the like.

Having described my invention, I claim:

1. A pavement composed of comminuted

stony material in the form of dust, intimately mixed with a suitable binder, and subjected to pressure.

2. A pavement composed of mechanically pulverized rock in the form of dust, intimately mixed with a bituminous binder, and spread and compacted upon the surface to be paved.

3. A pavement composed of mechanically 10 pulverized stony material in the form of dust, intimately mixed with from 12 to 18 per cent. of a bituminous binder and spread and compacted upon the surface to be paved.

4. A pavement composed of rock mechanically 15 pulverized to dust, intimately mixed with not less than 12 per cent. and not more than 16 per cent. of asphalt, spread and compacted upon the surface to be paved.

5. A pavement composed of pulverized 20 stony material such as stone, rock, sand or gravel, substantially 40 per cent. of which will pass a 200 mesh screen and approximately 90 per cent. of which will pass a 30 mesh screen, intimately mixed with bitumen, and spread and compacted upon the 25 surface to be paved.

6. A pavement composed of a mixture of 30 comminuted stony material and earthy material, both being in the form of dust, intimately mixed with a suitable binder and subjected to pressure.

7. A pavement composed of a mixture of 35 comminuted stony material and earthy material, both being in the form of a substantially dry dust, intimately mixed with a bituminous binder and spread and compacted upon the surface to be paved.

8. A pavement consisting of a tough and 40 tenacious wear resisting and traffic supporting material, composed solely of a mixture of stony material such as sand, gravel, rock or stone and earthy material such as soil, loam or clay, all pulverized to dust, and impregnated with from 12 to 20 per cent. of 45 asphalt.

9. The process of making a pavement 50 which consists in mixing pulverized stony material, such as sand, gravel, or stone, and pulverized earthy material, such as soil, loam or clay, substantially all in the form of fine dust, with not less than 12 per cent. of asphalt, spreading the mixture uniformly upon a prepared base and compacting it thereon.

55 10. The process of making a pavement, which consists in mixing stony material, pulverized to dust of such a fineness that at least 40 per cent. will pass a 200 mesh screen, with asphalt, the proportion of dust to asphalt being not more than 88 to 12 and not less than 80 to 20, spreading the mixture uniformly upon a prepared base and compacting it thereon.

11. The process of making a pavement,

which consists in mixing stony and earthy 65 material pulverized to dust to such a fineness that at least 40 per cent. will pass a 200 mesh screen, with asphalt, spreading the mixture uniformly upon a prepared base and compacting it thereon.

70 12. The process of producing paving material which consists in pulverizing disintegrated rock, stone, gravel, or sand to such a degree of fineness that 40 per cent. will pass a 200 mesh screen, and impregnating 75 the same with not less than 12 per cent. of asphalt.

13. The process of producing paving material which consists in mechanically comminuting stony and earthy material to dust, 80 mixing it with sufficient asphalt to form a nonflowing wear resisting and traffic supporting mass, spreading it uniformly upon a prepared base, and compacting it thereon.

14. The process of making a paving material, which consists in mixing pulverized 85 stony material such as sand, gravel or stone and disintegrated earthy material such as soil, loam or clay, with not less than 12 per cent. of asphalt, and compacting the same 90 under pressure.

15. The process of making a paving material, which consists in taking a natural earthy deposit, containing a large percentage of stony material, such as sand, gravel, or 95 the like, reducing it to such a degree of fineness that substantially half the total amount will pass a 200 mesh screen and at least 90 per cent. will pass a 30 mesh screen, intimately mixing it in that condition with not less than 12 per cent. of asphalt, and compacting the same under pressure.

16. The process of making a paving material, which consists in pulverizing stony 105 material such as sand, gravel, rock, and the like to that degree of fineness necessary for a thorough incorporation therewith and even distribution therethrough of a liquefied bituminous binder, impregnating it with such binder and then compacting it by pressure 110 whereby it becomes a tough malleable and durable material adapted for the purpose intended.

17. The process of making a paving material, which consists in pulverizing and 115 disintegrating stony material and earthy material to that degree of fineness necessary for a thorough incorporation therewith and even distribution therethrough of a liquefied bituminous binder, impregnating it with 120 such binder and then compacting it by pressure whereby it becomes a tough malleable and durable material adapted for the purpose intended.

18. The process of producing a homogeneous 125 wear resisting substance for paving purposes and the like, which consists in pulverizing friable stony materials to dust, and

incorporating the dust with a bituminous binder and compacting the mixture.

19. The process of producing a homogeneous wear resisting substance for paving or 5 other surfacing purposes, which consists in pulverizing friable earthy materials and soft stony particles to dust, and mixing the dust with a bituminous binder and compacting the mixture.

10 20. The process of producing a homoge-

neous wear resisting substance for paving or other surfacing purposes, which consists in simultaneously pulverizing friable stony materials and friable earthy material to dust and intimately mixing the same with a bituminous binder and compacting it. 15

In testimony whereof I have hereunto set my hand.

MICHAEL A. POPKESS.